

## 1

3,418,129

COLOR PHOTOGRAPHIC SILVER  
HALIDE EMULSION

Shiro Kimura and Makoto Yoshida, Odawara-shi, Japan, and Kazuya Sano, University Park, Pa., assignors to Fuji Shoshin Film Kabushiki Kaisha, Kanagawa-ken, Japan, a corporation of Japan  
No Drawing. Filed Dec. 9, 1964, Ser. No. 417,243  
Claims priority, application Japan, Dec. 27, 1963,  
38/70,436

The portion of the term of the patent subsequent to  
Aug. 22, 1984, has been disclaimed  
6 Claims. (Cl. 96—100)

## ABSTRACT OF THE DISCLOSURE

A color photographic silver halide emulsion containing as a coupler a compound of the formula:



wherein A is a coupling component having at least a member selected from the group consisting of ketomethylene group, pyrazolone nucleus, phenol nucleus, and naphthol nucleus, m is an integer from 2 to 7 and n is an integer from 6 to 14 when m is 2, 4, 5, 6 or 7 and n is 14 when m is 3.

This invention relates to light-sensitive silver halide emulsions for color photography and more particularly to a photographic silver halide emulsion containing a protective coupler.

In a conventional color photography using a coupler dispersed in a photographic emulsion, a method of making a coupler water-soluble and incorporating it as a form of an aqueous solution in the emulsion, and a method of making a coupler oil-soluble and incorporating it as a form of an organic solvent solution in the emulsion have occupied important positions. In the second method it is in particular important factors that the coupler has a higher solubility in an organic solvent in use for dispersing and a higher dispersibility during and after applied to a base as a light-sensitive material.

It is therefore an object of our invention to provide a novel coupler having a high solubility in a water-soluble solvent of high boiling point such as butyl phthalate, o-tolyl phosphate and butyl phosphate. Another object is to prevent the ununiformity of applying and the degradation of the final color picture caused by the deposition and aggregation of the coupler during and after the conventional process for producing light-sensitive material comprising, dispersing a coupler solution in a photographic emulsion, followed by applying the emulsion to a base and drying, or even after developing.

We have already found that a compound having the following general structure accomplishes these objects.



## 2

where A is a coupling component having at least one ketomethylene group, pyrazolone nucleus, phenol nucleus or a nucleus having phenolic hydroxyl group such as naphthol nucleus and n is an integer from 6 to 12.

Furthermore, we have found that a compound having the following structure not only accomplishes these objects, but represents an excellent property that is not given by the compound described as above,



where A is a coupling component having at least one ketomethylene group, pyrazolone nucleus, phenol nucleus or naphthol nucleus as above and m is an integer from 2 to 7, n is 14 when m is 3, and from 6 to 14 when m is 2, 4, 5, 6 and 7.

When n is less than 5, the diffusion of the coupler can be observed in the emulsion layer of light sensitive material and when m is 0 or 1, the insufficient solubility tends to cause a rapid deposition and aggregation during supercooling. When n is 15 or m exceeds 8, the solubility is too low. When n is 14, the solubility may be compared unfavourably with the case of less than this, but the compound can find a practical use in many cases, since the deposition by supercooling is very slow. For example, it is in a very advantageous position particularly when it is adapted for a light-sensitive material which should resist a severe thermal shock or when the coupling A has a property to promote crystallization.

Illustrative of such compounds of our invention is as follows:



To make clear that the compounds having the general structure have high solubilities, the comparison with couplers having a straight chain alkyl group is shown in Table 1.

TABLE 1.—COMPARISON BETWEEN BRANCHED CHAIN AND STRAIGHT CHAIN

| Compound                                            | (1) | (6)  | (2) | (7) | (3) | (8) | (4) | (9) |
|-----------------------------------------------------|-----|------|-----|-----|-----|-----|-----|-----|
| Melting point (° C.)                                | 64  | 102  | 125 | 168 | 91  | 143 | 80  | 129 |
| Gram dissolved in butyl phosphate, 100 g. at 25° C. | 5   | <0.1 | 21  | 4   | 70  | 29  | 45  | 5   |

The compounds 6-9 referred for the comparison are as follows:



The following examples illustrate the synthesis of the compounds of our invention and the application thereof to photographic light-sensitive material.

Synthesis of the Compound 1.—174 g. of methyl acrylate and 118 g. of propylamine were mixed in a reactor equipped with a cooler and the mixture was heated at 70° C. on a hot water bath to accomplish the reaction. The reaction product was distilled in *vacuo* to give 250 g. of methyl - 3 - propylaminopropionate as a fraction at 57° C./3 mm. Hg. 145 g. of the resulting methyl-3-propylaminopropionate and 120 g. of triethylamine were dissolved in 1.5 liters of ether, to which 246 g. of myristyl chloride was added dropwise with stirring and cooling by ice. After the addition, the mixture was stirred at room temperature for  $\frac{1}{2}$  hour and the resulting triethylamine chloride was filtered off. The ether solution was adequately washed with water, dried and distilled in *vacuo* to give 290 g. of methyl-3-(N-propylmyristamide)-propionate which boiled at 201-3° C./1.5 mm. 290 g. of the resulting ester and an alcoholic solution of 60 g. of potassium hydroxide were mixed, heated for 1 hour, refluxed and distilled off the alcohol. To the residual solution, were added 120 ml. of concentrated hydrochloric acid and 100 ml. of water to separate an acid, which was extracted with 1 liter of ether, dried by sodium sulfate anhydride and distilled to remove the ether therefrom. The product was recrystallized from methanol to give 205 g. of 3-(N-propylmyristamide)-propionic acid which melted at 45° C. 34 g. of this product was heated with 12 g. of thionyl chloride to some extent on a hot water bath to produce the corresponding oxychloride. All the resulting oxychloride was mixed with 23 g. of N-(2-aminoethyl)-1-hv-

droxy-2-naphthamide and 10 g. of pyridine, heated to condense, left standing for one night and the reaction mixture was transferred into a dilute hydrochloric acid to deposit an oily product. The oily product was washed with

water, crystallized with the addition of nitromethane and recrystallized from methanol to produce 3 g. of the final product which melted at 64° C.

The homologue thereof could be synthesized in the same manner as above but, in the case of the intermediate branched acid being oily at room temperature, it was employed as it was for the subsequent step after the step of removing ether.

Synthesis of the Compound 2.—3 - (N - propylcaprylic amide)-propionic acid was obtained as 210 g. of an oily product from 145 g. of methyl-3-propylaminopropionate, 120 g. of triethylamine, 163 g. of caprylic acid chloride and 60 g. of potassium hydroxide. 27 g. of the acid was reacted with 12 g. of thionyl chloride as in (1) and the product was mixed with 17.5 g. of 3-amino-1-phenyl-5-pyrazolone and 30 ml. of diethyl oxalate, followed by being heated on a hot water bath to evolve hydrogen chloride. The reaction product was added to 100 ml. of 50% aqueous methanol and left standing with cooling to crystallize. After filtered, the crystal was recrystallized from methanol to give 5 g. of the coupler which melted at 125° C.

The homologue thereof could be synthesized in the similar manner.

35      Synthesis of the Compound 3.—3-(N-butylpalmitamide)-propionic acid was produced by hydrolysis with 250 g. of potassium hydroxide of an ester obtained from 675 g. of methyl-3-butylaminopropionate, 1140 g. of palmitic acid chloride, 450 g. of triethylamine and 5 liters of ether, recrystallized from methanol to give 1150 g. of crystal which melted at 56° C. The acid thus resultant was adequately dried and 187 g. thereof was converted into the oxychloride with 64 g. of thionyl chloride. Then, 136 g. of 3-amino-1-(2,4,6-trichlorophenyl)-5-pyrazolone was suspended in 500 ml. of acetonitrile, to which the oxychloride was added dropwise with heating and stirring. The reaction proceeded with evolving hydrogen chloride gas. After 1 hour, the half amount of the acetonitrile was removed by distillation, 500 ml. of water was added thereto, and the mixture was left standing and cooling to crystallize, filtered, followed by recrystallization, thereby to give a crystal, 200 g. which melted at 91° C.

Any of the homologue of the compound could be synthesized in the similar manner. It could be synthesized in the same manner as in (2) but in the case the melting point of the product was low.

Synthesis of the Compound 4.—40 g. of the oxy-chloride obtained in the synthesis of the Compound 3 was added dropwise at room temperature to a suspension of 28 g. of 4-aminobenzoylaceto-2-methoxyanilide and 13 g. of triethylamine in 300 ml. of acetone, refluxed for a while, transferred into water to separate an oily product and the oily product was recrystallized from nitroethane and subsequently from ethanol. Yield: 15 g., M.P. 80° C.

The synthesis of aminobenzoylacetoanilide derivatives could be carried out in the same manner and, in addition, carried out as the following example.

70 Synthesis of the Compound 5.—3-(N-octylmyristamide)-propionic acid chloride was produced by reacting an acid obtained from 300 g. of methyl-3-octylamino-propionate, 200 g. of triethylamine, 344 g. of myristic acid chloride, 3 liters of ether and 85 g. of potassium hydroxide with 1.1 equivalent of thionyl chloride.

52 g. of ethyl-p-aminobenzoyl acetate was dissolved in 300 ml. of acetone, 30 g. of triethylamine was added thereto and 103 g. of the oxychloride was added dropwise with stirring at room temperature to deposit triethylamine hydrochloride with some condensate. After the addition, the reaction was continued for 1 hour, 100 ml. of water was added thereto and decanted. Mixed with ligroine in a small amount, crystallized, filtered and recrystallized from acetone. Yield: 20 g., M.P. 70° C.

20 g. of ethyl-p-(3-(N-octylmyristamide) propionamide)-benzoyl acetate was mixed with 5 g. of o-chloroaniline, reacted at 160° C. for 2/3 hour and, after cooled, crystallized by adding methanol. Recrystallized from ethanol to give 5 g. of a crystal which melted at 130° C.

Example 1

8 g. of the Compound 1 was dissolved in 20 g. of butyl phthalate with heating, the resulting solution was added to a mixed solution of 10 ml. of 5% saponin aqueous solution and 200 ml. of 5% gelatin aqueous solution, made emulsified and added to 500 g. of an emulsion of iodobromide. A film base coated by the resulting emulsion was dried, exposed, developed by the following developing solution, bleached and fixed.

|                                                 |      |
|-------------------------------------------------|------|
| 2-amino-5-N,N-diethylaminotoluene hydrochloride | 2.0  |
| Sodium sulfite                                  | 2.0  |
| Sodium carbonate                                | 20.0 |
| Potassium bromide                               | 2.0  |
| Water to 1 liter.                               |      |

The cyan image having the absorption maximum at 700 n.m. was obtained. The deposition and aggregation of the coupler could not be observed throughout the process and in the resulting color image and the Heiz value by ASTM was 9.1 at the maximum density. When the Compound 6 was treated in the same manner, the Heiz value reached 16.3 at the maximum density.

Example 2

6 g. of the Compound 2 was dissolved in 20 g. of butyl terephthalate and treated as in Example 1 thereby to obtain a magenta image having the absorption maximum at 545 n.m. The deposition and aggregation of the coupler could not be observed throughout the process and in the color image. The Heiz value by ASTM at the maximum density was 10.8, while that of the Compound 7 at the same condition was 50.8.

Example 3

10 g. of the Compound 3 was dissolved in 20 g. of butyl phthalate. This solution was poured into 150 ml. of 2% gelatin solution and then milled in a colloid mill to disperse. This dispersion was added to 100 g. of a positive emulsion. After coating on a film support, and dried, the film was exposed and processed in a developer of the following composition, after treating as usual, and was found to produce a satisfactory clear magenta image having the absorption maximum at 550 n.m.

|                                              |      |
|----------------------------------------------|------|
| N,N-diethyl-p-phenylenediamine hydrochloride | 2.0  |
| Sodium sulfite                               | 2.0  |
| Sodium carbonate                             | 20.0 |
| Potassium bromide                            | 2.0  |
| Water to 1 liter.                            |      |

The Heiz value by ASTM was 3.6 at the maximum density, while that of the Compound 8 was 79.3 at the same condition.

Example 4

10 g. of the Compound 4 was dissolved in a mixed solution of 18 g. of butyl phthalate and 2 g. of o-tolyl phosphate and treated as Example 1 thereby to produce a satisfactory yellow image having the absorption maxi-

mum at 442 n.m. The Heiz value by ASTM at the maximum density was 5.8, while that of the Compound 9 at the same condition was 46.8.

Example 5

8 g. of the Compound 5 was dissolved in a mixed solution of 15 g. of butyl phosphate and 5 g. of o-tolyl phosphate, dispersed in the similar manner to that described in Example 1 and processed in the developer described in Example 3 thereby to produce a satisfactory yellow image having the absorption maximum at 430 n.m. The Heiz value by ASTM at the maximum density was 5.7.

What we claim is:

1. A color photographic silver halide emulsion in which a compound represented by the following general structure is incorporated as a coupler:



25 where A is a coupling component having at least a member selected from the group consisting of ketomethylene group, pyrazolone nucleus, phenol nucleus, and naphthol nucleus, m is an integer from 2 to 7 and n is an integer from 6 to 14 when m is 2, 4, 5, 6 and 7 and n is 14 when m is 3.

30 2. The emulsion according to claim 1 wherein said coupler is a compound having the following formula:



35 3. The emulsion according to claim 1 wherein said coupler is a compound having the following formula:



45 4. The emulsion according to claim 1 wherein said coupler is a compound having the following formula:



5. The emulsion according to claim 1 wherein said coupler is a compound having the following formula:



6. The emulsion according to claim 1 wherein said coupler is a compound having the following formula:



**References Cited**

**UNITED STATES PATENTS**

3,337,344 8/1967 Kimura et al. ----- 96—100  
 3,135,609 6/1964 Klinger ----- 96—100

J. TRAVIS BROWN, *Primary Examiner.*

UNITED STATES PATENT OFFICE  
CERTIFICATE OF CORRECTION

Patent No. 3,418,129

December 24, 19

Shiro Kimura et al.

It is certified that error appears in the above identified patent and that said Letters Patent are hereby corrected as shown below:

In the heading to the printed specification, line 6, "Fuji Shoshin Film Kabushiki Kaisha" should read -- Fuji Shashin Film Kabushiki Kaisha --.

Signed and sealed this 2nd day of June 1970.

(SEAL)

Attest:

Edward M. Fletcher, Jr.

Attesting Officer

WILLIAM E. SCHUYLER, JR.

Commissioner of Patents